

## UNITED STATES PATENT OFFICE

2,545,076

REPEATEDLY IGNITABLE COMPOSITION  
ROD

Joseph Ellenbogen, London, England

No Drawing. Application April 8, 1946, Serial No.  
660,431. In Great Britain April 10, 1945

12 Claims. (Cl. 52—29)

1

This invention relates to repeatedly ignitable composition rods.

Various proposals have been made for the manufacture of such rods containing a combustible substance such as metaldehyde or nitrocellulose and an igniting mass which has sometimes formed the core of the rod, but these have suffered from the disadvantage that the core has tended to burn away more quickly than the combustible substance, so that after having been used a number of times difficulty is experienced in causing the rod to ignite. A further difficulty has also been experienced in that there has been a tendency for inorganic residues to accumulate on the exposed surface of the igniting mass.

It is an object of the present invention to overcome these disadvantages.

Accordingly, the present invention provides a repeatedly ignitable composition rod comprising a core containing an igniting substance and a hydrated inorganic salt having at least two molecules of water of crystallisation per molecule of salt and an outer layer containing a solid combustible substance such as metaldehyde and/or a nitrocellulose of the pyroxylin type.

The igniting substance in the core may contain an easily inflammable substance such as phosphorus and/or an oxidising agent such as potassium chlorate. If it contains both these components the rod may be struck on any rough surface, but if it contains only one of the components then it must be struck on a surface containing the other. Thus, if the core contains only an oxidising agent and a hydrated inorganic salt then the rod should be struck on a surface containing phosphorus.

The rod may also contain known combustion-retarding materials in addition to the hydrated inorganic salt. Examples of such combustion-retarding materials are chalk, zinc oxide and calcium plumbate.

The hydrated inorganic salts have two main functions. Firstly, they retard combustion of the core by evaporation of the water of hydration while the combustible mass is burning and the inorganic residue is lessened by the amount of water thus removed. Secondly, the salt hydrates melt at temperatures below that of the flame and render the core molten or plastic and some swelling of the mass occurs due to boiling away of the water of hydration. This second feature ensures that after extinguishing the flame, the core which then quickly solidifies just protrudes from the mass of combustible material and is ready for the next ignition.

2

If the composition contains both an easily inflammable substance and an oxidising agent the hydrated salt has the further function that in contradistinction to the compositions of United Kingdom Specification No. 500,219, it permits an excess of oxidising agent to be used, thereby avoiding a soft phosphorus and carbonaceous residue on the end of the core after ignition.

The hydrated inorganic salt may conveniently comprise from 5% to 50% by weight of the core.

Examples of hydrated inorganic salts which may be used are: tri-sodium phosphate dodecahydrate ( $Na_3PO_4 \cdot 12H_2O$ ), microcosmic salt

15  $(NaNH_4HP_4 \cdot 4H_2O)$

and alum ( $Al_2(SO_4)_3 \cdot 18H_2O$ ).

Examples of combustible substances which may be used are metaldehyde and nitrocellulose of 20 the pyroxylin type.

The bonding of the ingredients of the composition may be effected by the use of a gum such as gum arabic but since gums are themselves combustible and may cause undesired burning of the 25 easily inflammable substance and the oxidising agent it is preferred to use as a bonding agent an organo-silicon compound which polymerises to a resinous state. Any tendency towards undesired combustion is then stopped by the production of silica during the burning.

The rods of the present invention may be conveniently prepared by working up the ingredients into plastic masses and extruding these through nozzles. The core and the outer layer may if 35 desired be extruded through a composite nozzle in one operation.

The rod may be coated with an outer layer such as a lacquer or an asbestos composition.

The following are examples of rods according 40 to the invention. The parts are by weight.

1. A plastic mass for the core was prepared from an intimate mixture of 65 parts of potassium chlorate, 6 parts of alum, 3 parts of iron oxide, 14 parts of zinc oxide, 5 parts of gum arabic in the form of a 30% aqueous solution and 45 7 parts of cement. A plastic mass for the outer layer of combustible substance was prepared from an intimate mixture of 85 parts of metaldehyde and 15 parts of nitrocellulose of the pyroxylin type in the form of a 20% by weight solution in acetone. The two plastic compositions were extruded through a composite nozzle in one operation to form a rod. After evaporation of the solvents a firm rod was obtained which was then 50 55 coated with lacquer to control combustion of the

outer layer. The rod can be struck on a phosphorus surface.

2. The core consisted of an intimate mixture of 60 parts of potassium chlorate, 5 parts of potassium nitrate, 16 parts of microcosmic salt, 1 part of iron oxide, 10 parts of zinc oxide, 4 parts of gum arabic and 4 parts of cement. The outer layer of combustible substance consisted of an intimate mixture of 85 parts of metaldehyde and 15 parts of nitrocellulose of the pyroxylin type. The rod was produced as described in Example 1, and can be struck on a phosphorus surface.

3. The core consisted of an intimate mixture of 60 parts of potassium chlorate, 10 parts of sodium phosphate dodecahydrate ( $Na_3PO_4 \cdot 12H_2O$ ), 16 parts of silica, 5 parts of gum arabic, 1 part of iron oxide and 8 parts of cement. The outer layer of combustible substance consisted of an intimate mixture of 85 parts of metaldehyde and 15 parts of nitrocellulose of the pyroxylin type. The rod was produced as described in Example 1 and can be struck on a phosphorus surface.

4. The core consisted of an intimate mixture of 40 parts of potassium chlorate, 3 parts of red phosphorus, 20 parts of microcosmic salt, 1 part of iron oxide, 7 parts of zinc oxide, 4 parts of gum arabic and 25 parts of cement. The outer layer of combustible substance consisted of an intimate mixture of 85 parts of metaldehyde and 15 parts of nitrocellulose of the pyroxylin type. The rod was produced as described in Example 1 and can be struck on any rough surface.

5. The core was prepared by making an intimate mixture of 40 parts of potassium chlorate, 4 parts of phosphorus, 16 parts of zinc oxide, 15 parts of microcosmic salt, 1 part of iron oxide, 12 parts of cement and 12 parts of ethylortho-silicate, to which was then added 4 parts of 95% industrial alcohol, which caused resinification of the ethylortho-silicate. The outer layer of combustible substance consisted of an intimate mixture of 85 parts of metaldehyde and 15 parts of nitrocellulose of the pyroxylin type. The rod was produced as described in Example 1. After evaporation of the solvent a firm rod was obtained which was then coated with lacquer to control combustion of the outer layer. The rod can be struck on any rough surface.

I claim:

1. A repeatedly ignitable composition rod comprising a core containing a chlorate oxidizing agent together with a hydrated inorganic salt containing at least two molecules of water of crystallization per molecule of salt and an outer layer containing metaldehyde.

2. A repeatedly ignitable composition rod comprising a core containing a chlorate oxidizing agent and phosphorus together with a hydrated inorganic salt containing at least two molecules of water of crystallization per molecule of salt and an outer layer containing metaldehyde.

3. A repeatedly ignitable composition rod comprising a core containing phosphorus, a potassium chlorate oxidizing agent, together with a hydrated inorganic salt containing at least two molecules of water of crystallization per molecule of salt and an outer layer containing metaldehyde.

4. A repeatedly ignitable composition rod comprising a core containing phosphorus, potassium chlorate and a hydrated inorganic salt containing at least two molecules of water of crystallization per molecule of salt and an outer layer con-

taining metaldehyde, the proportion by weight of potassium chlorate being greater than that of phosphorus.

5. A repeatedly ignitable composition rod comprising a core containing potassium chlorate and a hydrated inorganic salt containing at least two molecules of water of crystallization per molecule of salt bonded by means of an organo-silicon compound, and an outer layer containing metaldehyde.

6. A repeatedly ignitable composition rod comprising a core containing potassium chlorate and alum and an outer layer containing metaldehyde and a nitrocellulose of the pyroxylin type.

7. A repeatedly ignitable composition rod comprising a core containing potassium chlorate, potassium nitrate and microcosmic salt and an outer layer containing metaldehyde and a nitrocellulose of the pyroxylin type.

8. A repeatedly ignitable composition rod comprising a core containing potassium chlorate and sodium phosphate dodecahydrate and an outer layer containing metaldehyde and a nitrocellulose of the pyroxylin type.

9. A repeatedly ignitable composition rod comprising a core containing potassium chlorate, red phosphorus and microcosmic salt and an outer layer containing metaldehyde and a nitrocellulose of the pyroxylin type.

10. A repeatedly ignitable composition rod comprising a core containing a chlorate oxidizing agent, together with a hydrated inorganic microcosmic salt containing at least two molecules of water of crystallization per molecule of salt and an outer layer containing metaldehyde.

11. A repeatedly ignitable composition rod comprising a core containing a chlorate oxidizing agent, together with alum containing at least two molecules of water of crystallization per molecule of salt and an outer layer containing metaldehyde.

12. A repeatedly ignitable composition rod comprising a core containing a chlorate oxidizing agent, together with sodium phosphate dodecahydrate, and an outer layer containing metaldehyde.

JOSEPH ELLENBOGEN.

#### REFERENCES CITED

The following references are of record in the file of this patent:

#### UNITED STATES PATENTS

| Number       | Name    | Date          |
|--------------|---------|---------------|
| 55 1,23,905  | Howse   | Feb. 20, 1872 |
| 1,941,621    | Ringer  | Jan. 2, 1934  |
| 2,138,378    | Johnson | Nov. 29, 1938 |
| 2,258,220    | Rochow  | Oct. 7, 1941  |
| 2,389,491    | Dunlap  | Nov. 20, 1945 |
| 60 2,408,398 | Johnson | Oct. 1, 1946  |

#### FOREIGN PATENTS

| Number  | Country       | Date          |
|---------|---------------|---------------|
| 3,424   | Great Britain | Nov. 26, 1869 |
| 10,994  | Great Britain | of 1901       |
| 329,796 | Great Britain | May 29, 1930  |
| 401,905 | Great Britain | Nov. 23, 1933 |
| 500,219 | Great Britain | Feb. 6, 1939  |

#### OTHER REFERENCES

H. D. Cogan: "Properties of Ethyl Silicate," Chemical and Engineering News, September 25, 1946, page 2501. (Copy in Patent Office Library.)